

W. G. ABBOTT, JR.  
INSOLE.  
APPLICATION FILED DEC. 4, 1915.

1,263,187.

Patented Apr. 16, 1918.

*Fig. 1.*



*Fig. 2.*



*Inventor*

William G. Abbott Jr.  
by Jas. H. Churchill  
atty.

# UNITED STATES PATENT OFFICE.

WILLIAM G. ABBOTT, JR., OF WILTON, NEW HAMPSHIRE, ASSIGNOR TO J. SPAULDING & SONS CO., OF ROCHESTER, NEW HAMPSHIRE, A COPARTNERSHIP COMPRISING MARION L. SPAULDING, OF BOSTON, MASSACHUSETTS, ROLAND H. SPAULDING AND HUNTLEY N. SPAULDING, BOTH OF ROCHESTER, NEW HAMPSHIRE, AND LEON C. SPAULDING, OF BUFFALO, NEW YORK.

## INSOLE.

1,263,187.

Specification of Letters Patent. Patented Apr. 16, 1918.

Application filed December 4, 1915. Serial No. 65,010.

To all whom it may concern:

Be it known that I, WILLIAM G. ABBOTT, Jr., a citizen of the United States, and a resident of Wilton, in the county of Hillsboro and State of New Hampshire, have invented an Improvement in Insoles, of which the following description, in connection with the accompanying drawings, is a specification, like characters on the drawings 10 representing like parts.

This invention relates to an insole for boots and shoes, and is an improvement upon an insole of flexible, substantially non-stretchable, chemically-treated fiber, whose 15 fibers are bonded together by a partial solution of the fibers themselves, and such as is shown and described in U. S. Letters Patent No. 1,135,217 granted April 13, 1915, to Huntley N. Spaulding.

20 Chemically-treated fiber sheets are made from a plurality of plies or layers of paper and are rendered pliable by moisture present in the fiber.

Chemically-treated fiber employed by me 25 is a product composed in whole or in part of cotton rags which are treated with suitable chemicals known to the trade to render the same substantially hard, non-stretchable, and non-compressible, and the fiber thus 30 treated is then treated with glycerin or other chemical in the presence of water to render the hard fiber pliable or flexible, the glycerin or other chemical incorporated in the fiber acting to retain a sufficient quantity 35 of water to insure the pliability desired.

The present invention has for its object to improve the chemically-treated fiber insole referred to, and to this end, the said insole is provided with a layer of linseed or other 40 drying oil which penetrates into the insole and then with a surface layer of pyroxylin or the like, whereby the moisture or other medium within the fiber for rendering the insole pliable is retained within the insole 45 by two layers, which repel external moisture, and one of which acts as a filler and lubricant to the fibers of the insole and also as a binder for the surface coating, which latter also forms an antifriction wearing 50 surface for the insole.

The particular features of this invention will be pointed out in the claims at the end of this specification.

Figure 1 represents in plan an insole embodying this invention, and

Fig. 2, a section on the line 2—2, Fig. 1, taken on an enlarged scale.

Referring to the drawing, *a* represents an insole for boots and shoes, which is such as shown and described in the patent referred to and composed of flexible, substantially non-stretchable chemically treated fiber containing moisture in sufficient quantity to impart to the insole the desired pliability, and in which the fibers of the insole are bonded together by a partial solution of the fibers 60 themselves.

The insole *a* is provided within it with a layer of linseed or other drying oil, which is indicated by the light broken lines *c*, and is also provided with a surface coating of pyroxylin or other varnish material, which is indicated by the heavy broken lines *b*, Fig. 2.

The layer *c* of oil is preferably baked or 70 subjected to heat to harden it before the pyroxylin coating *b* is applied.

The interior body portion *d* represents the natural condition of the chemically-treated fiber insole, such as shown in the patent referred to.

The oil layer *c* serves as a moisture-repelling layer and further acts as a filler and lubricant for the fibers of the chemically-treated insole; and serves as a binder for 85 the surface coating of pyroxylin to obtain a superior adhesion of the latter to the insole *a*, and to lessen the amount of the pyroxylin required, and further to retain the desired leather appearance and effect of 90 the chemically-treated fiber insole.

The pyroxylin coating *b* also serves as a moisture-repelling layer and increases the strength and firmness of the insole *a*. In addition, it provides the insole *a* with a 95 smooth, durable, antifriction wearing surface, which reduces to a minimum friction and heat created by movement of the foot of the wearer of a shoe provided with such insole, consequently reducing to a minimum 10

sweating of the feet and thereby providing a more comfortable and durable shoe for those persons whose feet perspire freely.

The oil layer may be formed within the 5 fiber by immersing the fiber sheet from which the insole is cut, in a bath of oil, and the surface coating may be applied by passing the sheet through a bath of pyroxylin.

It is preferred to use pyroxylin as the 10 surface layer or coating, but it is not desired to limit the invention in this respect, as other varnish materials, such as cellulose acetate, celluloid, resins, thickened oils, asphaltum, etc., may be used to advantage.

15 From the above description it will be seen that insoles of chemically treated fiber, whose fibers are bonded together by a partial solution of the fibers themselves and has within it a medium for rendering the 20 fiber pliable, when treated as above described, are superior to those made from untreated chemically-treated fiber, in that they retain their pliability and firmness for a relatively long time, as the medium which 25 makes the fiber pliable is retained within the fiber by two moisture repelling layers, their strength is increased, they are rendered

moisture-repellent, their life is prolonged, and they have a smooth and durable anti-friction wearing surface, which has the 30 property of reducing friction and heat and aids in providing a more comfortable and desirable boot or shoe for the wearer.

Claims.

1. An insole for boots and shoes composed of chemically-treated fiber of that character which has within it a medium for rendering said fiber pliable, said insole having within its body portion a layer of oil and at its surface a layer of pyroxylin, said 40 layers serving to retain the said medium within the insole.

2. An insole for boots and shoes composed of chemically treated fiber of that character which has within it a medium for rendering said fiber pliable, said insole having within its body portion a layer of oil and at its surface an anti-friction wearing layer of varnish material united with said layer of oil, said layers serving to retain the said 50 medium within the insole.

In testimony whereof, I have signed my name to this specification.

WILLIAM G. ABBOTT, JR.